

# United States Patent Office

2,693,278

Patented Nov. 2, 1954

1

2,693,278

## TREATMENT OF PYRRHOTITE ORES

Worth Martin Fitzsimmons, Stamford, Conn., assignor to American Cyanamid Company, New York, N. Y., a corporation of Maine

No Drawing. Application December 5, 1951,  
Serial No. 260,096

8 Claims. (Cl. 209—166)

This invention relates to the treatment of refractory pyrrhotite ores by froth flotation. More particularly, the invention relates to the treatment of pyrrhotite ores containing nickel and platinum values in addition to chromium oxide minerals.

In certain ores a refractory type of pyrrhotite occurs which cannot be readily floated with the ordinary sulfide collectors. The problem is particularly acute in certain nickeliferous pyrrhotite ores containing platinum associated with the pyrrhotite and which also have a large content of chromium oxide in the form of chromite. Such an ore deposit, for example, is found in the Philippine Islands.

According to the present invention, it has been found that if the ore is treated with an inorganic fluorine compound such as hydrofluoric acid, sodium fluosilicate and the like, the surface of the refractory pyrrhotite is altered and the pyrrhotite is then readily floated with conventional sulfide collectors such as xanthates, dithiophosphates and the like and a good separation is made from the gangue and chromite which is also present in the ore. It should be understood that the action of the fluorine compound affects the floatability of the pyrrhotite. This action has nothing in common, and should not be confused with the action of fluorine compounds in improving the floatation of various oxidized minerals. In fact, the action is actually substantially the reverse as the effect of the fluorine is not to enhance the floatation of the oxide minerals but, on the contrary, to activate the slow-floating sulfide, pyrrhotite. The exact mechanism is not fully known, but it is thought that one factor may be the presence of thin silicate coatings on pyrrhotite particles with which the fluorine compounds may react. Other factors may, however, play a part and it is therefore not desired to limit the invention to this particular theory of action of the fluorine compounds.

Application of the inorganic fluorine compound to the ore involves contact under acid conditions. Thus the ore may be conditioned with hydrofluoric acid and floatation then effected, a non-acid inorganic fluorine compound such as sodium fluosilicate may be used with sufficient acid, or the actual contact with the ore may be effected in the floatation circuit itself. Thus, for example, the ore can be conditioned with sodium fluosilicate and sulfuric acid added to the floatation cell or, alternately, the floatation may be effected with hydrofluoric acid. While it is not necessary that the fluorine compound and acid be both introduced in the conditioning step, best results are obtained under such circumstances, and this constitutes the preferred embodiment of the present invention.

The exact order of treatment is not rigidly limited but I prefer to condition first with sufficient acid to assure the requisite acidity in floatation; then condition the ore with the fluorine compound and additional acid, if required; followed by addition of the collector and another short additional conditioning. In some cases cleaning is necessary and additional amounts of reagents are sometimes needed.

When the refractory pyrrhotite ore is associated with chromite the latter is not floated in the first or sulfide float. The sulfide tail is deslimed, washed, and floated with a suitable chromite promoter in the normal manner. In other words, the present invention does not change the chromite floatation step but is directed solely to the sulfide floatation by which the pyrrhotite and its associated metal values are recovered.

Although the present invention is not limited to the

2

use of any particular sulfide collector, I have found that there is a considerable variation in the efficiency of different collectors, the best results being obtained with amyl xanthates. In a more specific aspect, therefore, the use of this collector is included. The invention will be described in greater detail in conjunction with the following examples. The metallurgical results for the examples are given in a table at the end.

### Example 1

A chromite ore containing a nickeliferous pyrrhotite with associated platinum values obtained from a Philippine deposit was ground with 5 lbs. per ton of sodium carbonate, and deslimed at 22% solids with 7 lbs. per ton of crude lignin sulfonate as a dispersant. The ore was then stage floated at a pH of 6.8 with 0.7 lb. per ton of potassium amyl xanthate, 10 lbs. per ton of sulfuric acid, 2 lbs. per ton of copper sulfate and 0.3 lb. per ton of a higher paraffin alcohol until no more sulfides were recovered. Total time of float was 60 minutes. The rougher concentrate was then conditioned for a short time with an additional 10 lbs. per ton of sulfuric acid and floated to produce a cleaner concentrate. The rougher tailing was conditioned with 3 lbs. per ton of an oil-soluble petroleum sulfonate and a chromite concentrate floated off which was cleaned once. The addition of the potassium amyl xanthate, frother, and sulfuric acid, during the sulfide float was made gradually in stages.

This procedure represents what may be termed conventional practice in the floatation of pyrrhotite. A good grade of concentrate was obtained, but the recovery of platinum group metals and nickel was very poor. The ore used in this example contained approximately 0.4 ounce per ton of platinum group metals, 0.5% nickel and 30%  $\text{Cr}_2\text{O}_3$ .

### Example 2

The ore of Example 1 was ground and deslimed as described above and conditioned at low (18%) solids, first with 10 lbs. per ton of sulfuric acid and then with 6 lbs. per ton of hydrofluoric acid, and finally, with 0.1 lb. per ton of potassium amyl xanthate and 0.03 lb. per ton of the higher alcohol frother. A sulfide float was effected in a much shorter time than in Example 1, approximately one-ninth as long. During the float there were added in two portions, at intervals, an additional 6 lbs. of hydrofluoric acid, 0.15 lb. per ton of the xanthate and 0.06 lb. per ton of the alcohol frother. The sulfide concentrate without cleaning showed approximately the same grade of platinum group metals and nickel, and approximately double the recovery. The sulfide tail was then treated on a Wilfley table to recover the chromite.

The difference in time of float was chosen because in the first example the pyrrhotite floated so slowly that the maximum floatation was used in order to obtain the best possible recovery. Obviously, the floatation time in Example 1 is so long that it would constitute an unattractive operation from the standpoint of cost. The test was made to give optimum possible recoveries so that the comparison would be under the best conditions for each operation.

### Example 3

The ore of Example 1 was ground, deslimed and conditioned first with 10 lbs. per ton of sulfuric acid then with 5 lbs. per ton of sulfuric acid and 2 lbs. per ton of sodium fluosilicate, and finally with 0.1 lb. per ton of potassium amyl xanthate. Froth floatation was then effected after adding 0.015 lb. per ton of the higher alcohol frother. The rougher float was effected in a series of five stages, the same amount of sulfuric acid, sodium fluosilicate, xanthate, and frother being added at each step. The sulfide concentrate was then cleaned and the rougher tailing deslimed, conditioned with 0.5 lb. per ton of oleic acid and floated to produce a rougher chromite concentrate. The latter concentrate was cleaned with the addition of 0.015 lb. per ton of the frother and 0.2 lb. per ton of oleic acid.

### Example 4

The procedure of Example 3 was followed, but the

## 3

ore was ground more finely, the grinding time being 50% greater. Also, in the cleaning step, additional sulfuric acid, sodium fluosilicate, potassium amyl xanthate and frother were used in amounts of 5.0, 2.0, 0.02 and 0.015 lbs. per ton, respectively.

## Example 5

The procedure of Example 4 was followed replacing the potassium amyl xanthate with potassium ethyl xanthate.

## Example 6

The procedure of Example 4 was followed but the potassium amyl xanthate was replaced with 0.2 lb. per ton of dicesol-dithio-phosphoric acid, and no frother was used since the promoter itself provided sufficient volume of froth for the purpose.

## Example 7

A Philippine dunite ore containing nickeliferous pyrrhotite and associated platinum group metals was ground and floated in four stages, each for five minutes. In each stage the pH ranged from 5.5 to 6.1. In the first stage there were 30 lbs. of sulfuric acid per ton, one pound per ton of secondary butyl xanthate and 0.06 lb. per ton of dicesol-dithio-phosphoric acid. The second two stages were effected each with the addition of 15 lbs. per ton of sulfuric acid, 0.5 lb. per ton of secondary xanthate and 0.02 lb. per ton of dicesol-dithio-phosphoric acid. In the last stage the amount of sulfuric acid was 10 lbs. per ton and 0.5 lb. per ton of potassium amyl xanthate was substituted for the secondary butyl xanthate. The ore analysed approximately 0.85% nickel with about 0.12 ounce per ton of platinum group metals.

## Example 8

The ore of Example 7 was conditioned first with 10 lbs. per ton of sulfuric acid, then with 5 lbs. per ton of sulfuric acid and 2 lbs. per ton of sodium fluosilicate, and finally with 0.10 lb. per ton of potassium amyl xanthate. Flotation was effected for two minutes with 0.015 lb. per ton of a higher paraffin alcohol frother. The conditioning with sodium fluosilicate, xanthate, and frother, was repeated in four more rougher stages, except that the amount of xanthate in each of these stages was reduced to 0.02 lb. per ton. The rougher concentrate was conditioned with 5.0 lbs. per ton sulfuric acid, 2.0 lbs. per ton sodium fluosilicate, 0.02 lb. per ton xanthate, and 0.015 lb. per ton higher paraffin alcohol frother, and then floated for two minutes for the production of a cleaner concentrate.

in the first flotation step 15 lbs. per ton of sulfuric acid were added and 5 lbs. per ton of sulfuric acid in each of the following four flotation steps, there being no conditioning outside of the flotation cell after each addition of acid. As in Example 9, the rougher concentrates were collected and assayed.

## Example 11

The procedure of Example 10 was followed except that 5 lbs. per ton of sulfuric acid were added to the pulp before conditioning to adjust its pH to 7.0, and the remaining 10 lbs. per ton of sulfuric acid added to the first flotation step. An additional 5 lbs. per ton of sulfuric acid were added in each of the succeeding flotation steps. As in Example 10, no conditioning was given after each float.

## Example 12

The procedure of Example 11 was followed except that there was no conditioning with sodium fluosilicate, nor was any sulfuric acid added to the flotation cell. Instead, 2.6 lbs. per ton of 48% hydrofluoric acid was added to the first step and a similar amount to each of the succeeding four stages. The rougher concentrates were collected and assayed.

The following table in which the recovery percentages are rounded off to the nearest whole number shows the comparative results of Examples 9 to 12, only recovery of platinum group metals and nickel being given. For comparison purposes, the calculated rougher concentrate of Example 4 is given.

| Ex. | Example | Percent Distribution-Sulfide Concentrate |        |
|-----|---------|------------------------------------------|--------|
|     |         | Platinum Group Metals                    | Nickel |
| 4   |         | 75                                       | 77     |
| 9   |         | 34                                       | 43     |
| 10  |         | 57                                       | 58     |
| 11  |         | 45                                       | 47     |
| 12  |         | 49                                       | 66     |

It will be noted from the above table that the presence of acid is essential. The use of an inorganic fluorine compound alone in Example 9 does not give any significant improvement over Example 1 in which no commercially significant fluorine compound was present. Practical, worthwhile improvements were obtained when both

| Ex.            | Assay                        |             | Percent Distribution-Sulfide Concentrate |        |                                |       | Chromite Concentrate           |               |                |
|----------------|------------------------------|-------------|------------------------------------------|--------|--------------------------------|-------|--------------------------------|---------------|----------------|
|                | Pt Group Metals, oz. per ton | Ni, Percent | Pt Group Metals                          | Nickel | Cr <sub>2</sub> O <sub>3</sub> | Conc. | Cr <sub>2</sub> O <sub>3</sub> |               | Ratio of Conc. |
|                |                              |             |                                          |        |                                |       | Grade, Percent                 | Rec., Percent |                |
| 1              | 6.1                          | 11.68       | 29.7                                     | 35.4   | 0.3                            | 64.2  | 44.69                          | 55.6          | 2.7            |
| 2 <sup>a</sup> | 7.08                         | 10.24       | 62.3                                     | 67.1   | 1.5                            | 27.9  | 48.64                          | 56            | 2.7            |
| 3              | 11.2                         | 9.71        | 56.4                                     | 39.3   | 0.9                            | 49.5  | 45.34                          | 68.2          | 2.2            |
| 4              | 9.86                         | 15.03       | 69.5                                     | 73.1   | 0.9                            | 35.8  | 48.66                          | 66.6          | 2.3            |
| 5              | 11.53                        | 20.42       | 53.9                                     | 62.9   | 0.2                            | 63.8  | 49.25                          | 58.3          | 2.7            |
| 6              | 9.96                         | 19.34       | 45.2                                     | 66.5   | 0.3                            | 64.5  | 48.37                          | 51.7          | 3.1            |
| 7 <sup>b</sup> | 3.5                          | 55.8        |                                          |        | 7.5                            |       |                                |               |                |
| 8              | 2.64                         | 16.37       | 41.6                                     | 37.2   |                                | 51.4  |                                |               |                |

<sup>a</sup> Rougher flotation, no cleaning.

<sup>b</sup> 4.5 for the first rougher concentrate, 2.5 for the next two and 2.4 for the last, averaging 3.5.

## Example 9

The ore of Example 1 was conditioned with 2 lbs. per ton of sodium fluosilicate and then with 0.1 lb. per ton of potassium amyl xanthate. Flotation was then effected with 0.015 lb. per ton of a higher alcohol frother. The tailing was then conditioned with an additional 2 lbs. per ton of sodium fluosilicate and 0.02 lb. per ton of potassium amyl xanthate, flotation being again effected with the same amount of higher alcohol frother. This second step was then repeated four times. The total rougher concentrate was collected and assayed.

## Example 10

The procedure of Example 9 was followed, except that

acid and fluorine compound were present even though there was no conditioning of the ore with the two materials prior to flotation. However, the results fall considerably short of those obtainable by one of the preferred procedures in Example 4 where the fluorine compound and acid were used in conditioning the ore before flotation took place.

This application is a continuation-in-part of application S. N. 246,715, now abandoned.

I claim:

1. As an improved process of floating a refractory pyrrhotite from an ore which contains as its principal values nickeliferous pyrrhotite containing platinum group metals associated with the pyrrhotite, the improved

process which comprises subjecting the said ore under acid conditions to froth flotation in contact with a soluble inorganic fluorine-bearing compound and a sulfide collector to produce a concentrate relatively rich in nickeliferous pyrrhotite and platinum group metals and a tailing relatively poor in pyrrhotite.

2. The process of claim 1 in which the sulfide collector is a xanthate.

3. As an improved process of floating refractory pyrrhotite from an ore which contains as its principal values nickeliferous pyrrhotite containing platinum group metals associated with the pyrrhotite, the improved process which comprises conditioning the said ore under acid conditions with a soluble inorganic fluorine-bearing compound and subjecting the so conditioned ore to froth flotation under acid conditions, in the presence of a sulfide collector to produce a concentrate relatively rich in nickeliferous pyrrhotite containing platinum group metals and a tailing relatively poor in pyrrhotite.

4. The process of claim 3 in which the sulfide collector comprises a xanthate.

5. The process of claim 4 in which the sulfide collector comprises an alkaline metal amyl xanthate.

6. The process of claim 3 in which the inorganic fluorine compound is hydrofluoric acid.

7. The process of claim 3 in which the said ore contains as its principal values a chromite and a nickeliferous pyrrhotite containing platinum group metal associated with the pyrrhotite.

8. The process of claim 7 in which the chromite is subsequently recovered from the said tailings.

References Cited in the file of this patent

UNITED STATES PATENTS

| Number    | Name           | Date          |
|-----------|----------------|---------------|
| 2,412,217 | Havens         | Dec. 10, 1946 |
| 2,556,215 | Queneau et al. | June 12, 1951 |

OTHER REFERENCES

A. I. M. M. E. Technical Paper 1074, © 1939, printed in Mining Technology, vol. 3, 1939 (16 pages). Copy in Division 55.